

1

3,515,543

## HAFNIUM ALLOYS

Peter Harlow Morton, Solihull, and Peter Vincent McDonald Clark, Moseley, Birmingham, England, assignors to Imperial Metal Industries (Kynoch) Limited, Witton, Birmingham, England, a corporation of Great Britain

No Drawing. Filed Nov. 28, 1966, Ser. No. 597,205  
Claims priority, application Great Britain, Dec. 2, 1965,

51,235/65

Int. Cl. C22c 31/00

U.S. Cl. 75—134

7 Claims

### ABSTRACT OF THE DISCLOSURE

Hafnium-base alloys suitable for nuclear reactor control rods consist of, by weight, at least one of the beta-stabilising elements zirconium 5–30% and niobium 15–30%, up to 2% in total amount of at least one of the beta-stabilising elements chromium, molybdenum, nickel and iron, up to 0.5% silicon, and up to 2% in total amount of one or both of the alpha stabilising elements tin and aluminium, the total content of alloying elements being not greater than 30%, balance hafnium and impurities.

This invention relates to hafnium alloys.

Hafnium is used for control rods in nuclear reactors because of its high neutron absorption coefficient. However, there are occasions when a material with a lower coefficient but having a comparable or better strength and corrosion resistance is required.

According to the present invention, a hafnium-base alloy consists of, by weight, one or both of the beta stabilising elements, zirconium 5–30% and niobium 15–30%, 0–2% in total of one or more of the beta stabilising elements, chromium, molybdenum, nickel and iron, 0–0.5% silicon, 0–2% in total of one or both of the alpha stabilising elements, tin and aluminium, the total content of alloying elements being not greater than 30%, balance hafnium and impurities.

The term "impurities" as used herein excludes zirconium which is frequently present in hafnium up to about 4%.

The preferred ranges of composition are 5–25% zirconium, 15–25% niobium, 0.1–2% in total of one or more of chromium, molybdenum, nickel and iron, 0.01–

2

0.5% silicon, 0.1–2% in total of one or both of tin and aluminium. Preferably, the total content of alloying elements should be between 10 and 30%.

The effect of the beta stabilising elements is to strengthen hafnium; the alpha stabilising elements, whilst having little effect on strength when added alone, generally improve the properties of the beta stabilised alloy.

The addition of niobium and zirconium reduces the neutron absorption coefficient and improves tensile strength. Niobium is considerably more effective in this latter respect than zirconium when only one of these elements is present. When both are present, the tensile strength is more than double that of commercially pure hafnium whilst the ductility is reduced by only a small amount. Additions of small amounts of the other beta stabilising elements, chromium, molybdenum, nickel, iron and silicon and of the alpha stabilising elements, tin and aluminium, further improve the tensile properties.

Corrosion resistance depends upon the alloying elements added and the amounts present. Zirconium has little effect on the excellent corrosion resistance of hafnium but niobium tends to increase the amount of surface film formed on exposure to high temperature pressurised steam. Below 15% niobium there is an appreciable loss of corrosion resistance.

The corrosion resistance of the alloys of the invention was determined by exposing cleaned bright samples to steam at a pressure of 100 atmospheres and at a temperature of 400° C. for 72 hours. The corrosion behaviour was compared by the appearance of the surface of the samples in accordance with the following classification.

(A) Glossy, bright, thin, adherent film (including interference films).  
(B) Glossy, bright, thick, adherent film.  
(C) Mottled appearance with dull patches or streaks which are usually powdery.  
(D) Dull but adherent film.

It is important that the film should be adherent with no tendency to powder or to flake off. In the above classification, class (A) has the best corrosion resistance.

The tensile properties and corrosion resistance of a number of alloys in accordance with the invention are shown by way of example in the table in comparison with pure hafnium. In the table, the abbreviation  $4\sqrt{A}$ , used in connection with the elongation values, refers to the gauge length of test pieces, that is, a gauge length equal to four times the square root of the area of the cross-section of the test piece. The corrosion resistance was determined in accordance with the above classification.

TABLE

| Alloy                | Composition<br>(analysed) | Corrosion<br>resistance | 0.2% P.S.<br>t.s.i. | U.T.S.<br>t.s.i. | Elongation,<br>percent<br>on $4\sqrt{A}$ |
|----------------------|---------------------------|-------------------------|---------------------|------------------|------------------------------------------|
| Unalloyed<br>hafnium | -----                     | -----                   | 15.6                | 25.3             | 26                                       |
| Zr1.....             | 10% Zr.....               | A                       | 11.8                | 28.6             | 24                                       |
| Zr2.....             | 20% Zr.....               | A                       | 16.0                | 20.4             | 30                                       |
| Zr3.....             | 30% Zr.....               | A                       | 12.8                | 28.9             | 23                                       |
| Nb5.....             | 20% Nb.....               | B                       | 43.6                | 47.3             | 28                                       |
| Nb6.....             | 25% Nb.....               | D                       | 46.1                | 49.9             | 23                                       |
| T1.....              | 15Nb-10Zr.....            | D                       | 53.4                | 58.4             | 21                                       |
| Q1.....              | 15Nb-10Zr-0.8Sn.....      | C                       | 57.0                | 62.4             | 16                                       |
| T7.....              | 20Nb-0.8Sn.....           | D                       | 44.8                | 49.5             | 20                                       |
| T8.....              | 25Nb-0.8Sn.....           | D                       | 46.7                | 51.6             | 25                                       |
| T3.....              | 25Zr-0.5Mo.....           | A                       | 13.7                | 30.6             | 23                                       |

We claim:

1. A hafnium-base alloy consisting of, by weight, at least one beta stabilising element selected from the group consisting of zirconium 5-30% and niobium 15-30%; up to 2% in total of at least one beta stabilising element selected from the group consisting of chromium, molybdenum, nickel and iron; up to 0.5% silicon; up to 2% in total of at least one alpha stabilising element selected from the group consisting of tin and aluminium, the total content of alloying elements being not greater than 30%; balance hafnium and impurities.
2. A hafnium-base alloy according to claim 1 in which the total content of alloying elements is between 10 and 30%.
3. A hafnium-base alloy according to claim 1 containing 5-25% zirconium.

10

5

15

4. A hafnium-base alloy according to claim 1 containing 15-25% niobium.
5. A hafnium-base alloy according to claim 1 containing 0.1-2% in total of one or more of chromium, molybdenum, nickel and iron.
6. A hafnium-base alloy according to claim 1 containing 0.1-2% in total of one or both of tin and aluminium.
7. A hafnium-base alloy according to claim 1 containing 0.01-0.5% silicon.

#### References Cited

##### UNITED STATES PATENTS

- |           |         |                |       |        |
|-----------|---------|----------------|-------|--------|
| 2,234,969 | 3/1941  | Hensel et al.  | ----- | 75-134 |
| 2,810,640 | 10/1957 | Bolkcom et al. | ----- | 75-134 |

RICHARD O. DEAN, Primary Examiner